

## UNITED STATES PATENT OFFICE

2,115,749

## METHOD OF COATING FERROUS ARTICLES

Michael M. Rubin, Warren, Ohio, assignor to  
The Thomas Steel Company, Warren, Ohio, a  
corporation of Ohio

No Drawing. Application May 8, 1936,  
Serial No. 78,724

2 Claims. (Cl. 204—8)

This invention relates, as indicated, to methods of applying alloy coatings to ferrous articles, but has reference more particularly to the production of a brass coating on such ferrous articles as 5 wire and strip.

It has heretofore been proposed to form such coatings on ferrous articles by electrodeposition on the articles of the alloy, or by immersing the articles to be coated in a molten bath of the alloy. These methods have generally proven unsatisfactory, as they do not result in the production of a coating of uniform thickness and homogeneity or one that adheres to the base metal with sufficient tenacity to render the article 10 capable of being subjected to bending and other fabricating operations.

It is an object of the present invention to provide a method whereby ferrous articles, such as wire and strip, are coated with a bright, uniform, closely adherent coating of brass.

20 A further object of the invention is to provide a method of the character described which is preferably continuous in character, but which may, if desired, consist of separate, discontinuous steps or operations.

25 To the accomplishment of the foregoing and related ends, said invention, then, consists of the steps hereinafter described and particularly pointed out in the claims, the following description setting forth in detail one approved method 30 of carrying out the invention, such disclosed method, however, constituting but one of the various ways in which the principle of the invention may be used.

35 The method, broadly stated, consists in separately electrodepositing on the ferrous article, such as strip or wire, the metals forming the alloy or brass coating, and subsequently heat treating the coated article in a controlled atmosphere free from oxidizing gases.

40 In providing, for example, a commercial yellow brass coating on steel strip, I first deposit on the strip, by any of the approved methods of electro-plating, a coating of copper in an amount of about .1 oz. of copper per square foot of strip surface. I then deposit upon the copper coating thus formed, and in a similar manner, a coating of zinc in an amount of about .05 oz. per square foot of surface. I then pass the article, 45 thus provided with coatings of copper and zinc, through a controlled atmosphere, free from oxidizing gases, such as oxygen, carbon dioxide, etc., and having a temperature of about 700° F. to about 1500° F., and maintain the article at this 50 temperature from about 10 to about 30 minutes, 55

or for a period of time sufficient to permit a complete alloying of the coatings to form yellow brass, the period of time of heating depending upon the thickness of the separate coatings and the specific temperatures employed.

5 The brass coating, thus formed, is bright, of uniform thickness, homogeneous in character, and adheres to the ferrous base metal with a tenacity sufficient to render the article capable of being subjected to bending and various other 10 operations employed in fabricating the article.

Because of the ease and accuracy with which the electrodeposition of the individual metals, copper and zinc in this instance, may be controlled, the composition of the alloy coating may 15 be more closely and readily controlled than in the case of the method previously referred to in which an alloy coating is directly deposited on the base metal. Thus, coatings of any of the well-known forms of brass may be obtained by 20 merely varying the thickness of the coating of each of the individual metals, since in this manner any desired ratio of such metals may be obtained, and it is unnecessary to change the composition of the plating baths. The method, as 25 thus described, is preferably carried out in a continuous manner, that is by causing the ferrous strip to travel continuously and uninterruptedly through the separate plating baths and the controlled heated atmosphere, but it will be understood that the method may also be carried out in a series of separate or discontinuous steps or operations. It will be also understood that instead of first depositing the copper, as described, 30 the base metal may be initially coated with zinc. 35

Other modes of applying the principle of my invention may be employed, instead of the one explained, change being made as regards the method herein disclosed, provided the step or steps stated by any of the following claims or the equivalent of such stated step or steps be employed.

I therefore particularly point out and distinctly claim as my invention:

1. The method of coating ferrous strip and the like which comprises continuously moving and consecutively subjecting the strip to the action of a copper electro-plating bath to form a coating of copper directly thereon and then to the 50 action of a zinc electro-plating bath to form a coating of zinc directly on the copper and finally to heating at a temperature of about 700° F. to about 1500° F. in a non-oxidizing atmosphere, 55 for from about 10 to about 30 minutes, whereby

to cause an alloying of the copper and zinc to form a non-peeling coating of brass.

2. The method of coating ferrous strip and the like which comprises consecutively subjecting the strip to the action of a copper electro-plating bath to form a coating of copper directly thereon and then to the action of a zinc electro-

plating bath to form a coating of zinc directly on the copper and finally to heating at a temperature of about 700° F. to about 1500° F. in a non-oxidizing atmosphere whereby to cause an alloying of the copper and zinc to form a non-peeling coating of brass. 5

MICHAEL M. RUBIN.